

## 1

3,105,762

**PHOTOGRAPHIC OVERCOATING**

John F. Byrne and Philip F. Kurz, Columbus, Ohio, assignors, by mesne assignments, to Minneapolis-Honeywell Regulator Company, a corporation of Delaware  
 No Drawing. Filed May 25, 1960, Ser. No. 31,555  
 4 Claims. (Cl. 96—67)

The present invention relates broadly to photosensitive compositions and more particularly to photographic compositions of the "print-out" type. The invention relates specifically to an overcoating composition to be applied to such photosensitive base compositions which will improve the "print-out" characteristics of the photosensitive compositions. The term "print-out" refers to that type of photosensitive substance upon which a visible image is obtained after an exposure to light or other electromagnetic radiation has been initially utilized to form a latent image, the visible image being obtained simply by an additional exposure to such radiation, normally at a somewhat lower intensity. This additional exposure is known as "latensification" and is general in its application, including exposing the area upon which the initial image was formed as well as the surrounding background area to an added amount of radiation. The further discussion of the latensification type photographic compositions can be found in the application of Troy A. Scott, No. 737,758, filed May 26, 1958, and assigned to the same assignee as the present invention.

Photographic compositions of the "print-out" type showing the latensification have found use in oscillographic recording and the like. The invention, as disclosed in the Scott application noted above, is particularly adaptable to this type of recording in that it shows a sensitivity equivalent to 200,000 lineal inches per second capability. Utilizing the overcoating of the present invention, the over-all properties of the photosensitive material are enhanced and a decidedly superior product results.

We have found that the trace density and the stability of the trace of the invention of the aforementioned application can be improved utilizing the method of the current application. In addition, the overcoating of the present invention provides a water proofing that is desirable to reduce the need for special storage and handling conditions prior to use.

The overcoating is a necessary adjunct to the base of photosensitive material for two reasons. First, a water proofing coating is highly desirable to reduce the need for special storage and handling conditions, and second, the trace definition of exposed paper is improved considerably by the use of the overcoating. The exact mechanism by which the improved definition is obtained is not known.

The polymer utilized to act as a water proofing agent and a carrier for the other constituents of the overcoating, a cupric halide and a formate, can be any of a number of commercially available polymers. Of course, it must be an effective water barrier and not affect the sensitivity of the photographic compositions. While other materials prove usable, the most desirable all-around properties have been found with vinyl acetate polymer emulsions.

In order to more particularly set out the features of the present invention, specific examples of preparation technique are presented hereinbelow.

**EXAMPLE I**

In accordance with the preferred embodiment of the present invention, the following preparation was prepared.

## 2

*Preparation of Silver Nitrate Solution*

| Compound:                                               | Amount             |
|---------------------------------------------------------|--------------------|
| AgNO <sub>3</sub>                                       | 170 gr. (1.0 mol). |
| H <sub>2</sub> O (distilled)                            | 1000 cc.           |
| NH <sub>3</sub> (20-30% aqueous solution, sp. gr. 0.90) | 400 cc.            |

The silver nitrate was weighed and dissolved in the prescribed amount of distilled water. Then the ammonia solution was added with stirring until the solution cleared as the precipitate of silver oxide formed by the first added portions of the ammonia was redissolved.

*Potassium Halide Solution*

| Compound:                    | Amount                |
|------------------------------|-----------------------|
| KI                           | 1.66 gr. (0.010 mol). |
| KBr                          | 143 gr. (1.20 mol).   |
| H <sub>2</sub> O (distilled) | 300 cc.               |

The potassium iodide was weighed carefully in order to insure precise control over the iodide content of the resultant silver halide mixture. The potassium halides were dissolved in the prescribed amount of water contained in a two-liter beaker which was set in a water-ethylene glycol bath. The bath was heated on a hot plate to about 70°-80° C. The solution of potassium halide was stirred mechanically with a stainless steel stirrer.

*Preparation of Silver Bromo-Iodide*

When the halide solution was hot (70° to 80° C.) the ammoniacal silver nitrate solution was added slowly in a steady stream to the reaction vessel. This was done by pouring the silver solution slowly into a funnel to the outlet of which has been fused a short length (about 4 inches) of capillary tubing. The capillary jet delivered the silver solution at a rate of about 30 cc. per minute, so that the addition of silver was completed in about 50 minutes. While the iodide reacts preferentially because of its being less soluble than the silver bromide, there may be considerable co-precipitation so that silver iodide is trapped in silver bromide crystals with the result that strained crystals of high sensitivity are formed.

Ammonia and potassium bromide act as solvents for the silver halides formed and promote crystal growth. Thus, in the presence of these solvents, the smaller silver halide crystals may dissolve and be re-deposited on the surfaces of larger crystals by a process known as Ostwald ripening. This process can occur during the slow precipitation step. The mixture was stirred vigorously with a mechanical stirrer during the precipitation period.

After the precipitation step, the silver halide mixture was filtered by suction on a Büchner funnel and was washed five times with distilled water. It is not normally necessary to dry the silver halides after filtering and washing.

In addition to the silver bromo-iodide, cadmium iodide was employed to increase the print-out effect and to assist in suppressing background during latensification.

| Compound:                                                       | Amount  |
|-----------------------------------------------------------------|---------|
| Silver halide (as prepared hereinabove)                         | gr. 100 |
| Cadmium iodide                                                  | gr. 5   |
| Water (distilled)                                               | cc. 50  |
| Hydroxyethyl starch (30% hydroxyethyl starch in water solution) | gr. 67  |

The ingredients listed above with the exception of the hydroxyethyl starch solution were placed in a pint porcelain jar of a ball mill containing 200 grams of one-half inch porcelain pebbles. The bottle was rotated at about 60 r.p.m. for a period of one hour. The hydroxyethyl starch was then added and the mixture ball-milled for

another one hour, after which time a homogeneous mixture resulted. The mixture described above had a consistency which was found readily adaptable for making flow-coated papers.

In this connection various application techniques may be employed, such as transfer roller coating, dip coating using an air-knife to wipe off the excess upon emergence from the bath, or by conventional spreading using a doctor knife to control the thickness of the film. Although the thickness of the coatings to be applied to paper or other supports is dependent on the characteristics desired in the end product, it has been found that if the composition disclosed above is applied in layers calculated to be in the range of about 0.5 mil in thickness a useful product results. As the thickness of the wet film is difficult to measure, it is somewhat easier to use the weight per unit area of solids deposited as a reference. About 1 gram of solids per square foot of the dried film appears to be satisfactory. The critical features are that the coating be uniform, flexible, and adherent to the base material. After application to the base plate, the coating was permitted to dry.

#### Overcoating Mixture

Following the above steps we have found that a coating of the following materials provide a surface sensitizing, water proofing effect.

|                                |         |      |
|--------------------------------|---------|------|
| Vinyl acetate polymer emulsion | gallons | 1    |
| Distilled water                | do      | 1    |
| Cupric chloride solution       | ml.     | 180  |
| Sodium formate solution        | ml.     | 3600 |
| Total                          | gallons | 3    |

The above components are prepared as follows: Vinyl acetate polymer emulsion of approximately 50% solid is used as received. We have found that vinyl acetate polymer emulsion supplied by B. F. Goodrich Chemical Company under their designation Geon Latex (970X11) is especially well suited for this purpose.

The cupric chloride solution is prepared by dissolving 25 grams of cupric chloride dihydrate ( $CuCl_2 \cdot 2H_2O$ ) in 500 ml. of water. Use 60 ml. of this solution for each gallon of overcoating mixture compounded.

The sodium formate solution is prepared by dissolving 400 grams of sodium formate ( $HCOONa$ ) in 1,600 ml. of water. Use 1,200 ml. of this solution for each gallon of overcoating mixture to be compounded. The cupric chloride solution and the formate solution are then combined into one solution in the proportion tabulated above, 180 ml. cupric chloride to 3,600 ml. of formate solution.

A blending of the above materials into a common solution must be made in the order in which they are designated above. That is, the vinyl acetate polymer emulsion is first diluted by addition of the distilled water and then the cupric chloride solution is added to the mixture of the vinyl acetate polymer emulsion and the distilled water. Unless these steps are followed in the order indicated there is a possibility of breaking the dispersion of the vinyl acetate polymer emulsion and water. Blending should be accomplished with sufficient stirring to insure a homogeneous end product.

This mixture is applied over the main coating to increase image density and stability. An extremely thin coating suffices. Measurements of coating weight indicate that about 0.3 gram of solid per square foot should be present in the overcoat. This overcoating may be applied in the same manner as noted above. That is, transfer roller coating, dipcoating using an air knife to wipe off the excess upon emergence from the bath, or by conventional spreading using a doctor knife to control the thickness of the film.

#### EXAMPLE II

The pre-treatment of the paper to provide a photosen-

sitive coating was the same as in Example I. The overcoating for Example II was prepared as follows:

|                                |         |      |
|--------------------------------|---------|------|
| Vinyl acetate polymer emulsion | gallons | 1    |
| Distilled water                | do      | 1    |
| Cupric bromide solution        | ml.     | 180  |
| Potassium formate solution     | ml.     | 3600 |
| Total                          | gallons | 3    |

The above components are prepared in the same manner as indicated in Example I with the exception of the potassium formate solution and cupric bromide solution. The potassium formate solution is prepared by dissolving 494 grams of potassium formate into 1,600 ml. of  $H_2O$ . Use 1,200 ml. of this solution for each gallon of overcoating mixture to be compounded. The cupric bromide solution is prepared by dissolving 33 grams of cupric bromide into 500 ml. of water. Use 60 ml. of this solution for each gallon of overcoating mixture. The blending of the materials of the overcoating mixture is the same as in Example I. That is, the vinyl acetate polymer emulsion is first diluted by addition of the distilled water and then the mixture of cupric bromide solution and potassium formate solution, blended together, are added to the mixture of the vinyl acetate polymer emulsion and distilled water. The overcoating is applied by any of the methods of Example I.

#### EXAMPLE III

The solutions in Example III including the photosensitive coating initially applied to the paper are prepared in the same manner as in Example I. The overcoating mixture is as follows:

|                                |         |      |
|--------------------------------|---------|------|
| Vinyl acetate polymer emulsion | gallons | 1    |
| Distilled water                | do      | 1    |
| Cupric chloride solution       | ml.     | 180  |
| Ammonium formate solution      | ml.     | 3600 |
| Total                          | gallons | 3    |

The above components were prepared in the same manner as indicated in Example I with the exception of the formic acid solution. The ammonium formate solution was prepared by dissolving 350 grams of ammonium formate into 1,600 ml. of water. Use of 1,200 ml. of this solution for each gallon of overcoating mixture to be compounded. Again, as in the above examples, the cupric chloride solution is added to the formate solution to comprise one gallon of the over-all mixture. The blending of the vinyl acetate emulsion, the distilled water, and the cupric chloride-formate solution follows the same procedures outlined above. The mixture is applied in the same manners as in Examples I and II with a coating thickness equivalent to that previously noted, 0.3 gram of solid per square foot.

The sensitive material and overcoating prepared in accordance with the examples hereinabove was yellow in color, and upon the desired exposure to light, a uniform medium dark brown image or trace having extremely uniform and fine edge definition was formed. Sensitive papers, prepared according to this process, were capable of writing speeds equivalent to more than 200,000 inches per second when illuminated from a source having an intensity of about 100,000 candles per square centimeter. Various commercially available high intensity light sources may be employed for producing the trace image such as the Osram lamp, the lamp being employed as specified in the aforementioned specification of Mahoney et al. The Osram lamp is manufactured by Osram, Munich, West Germany, and identified as their model HBO-107/1, high pressure mercury lamp.

The stabilizing overcoat of the invention increases the trace density and improves the stability of the trace and accordingly prevents fading upon post exposure to ambient light. Coated paper produced using the overcoating

composition of the invention produced traces that were much more dense than those traces on identically coated paper without the overcoating. In addition, the traces produced on paper having the overcoating of the invention were more stable than those traces on non-overcoated paper on prolonged exposure to fluorescent light of desk level intensity (50-100 fc.).

Having thus described our invention, what is claimed is:

1. A photosensitive silver halide print-out emulsion having thereon an overcoating consisting essentially of a water insoluble vinyl acetate polymer emulsion carrier and including as a constituent thereof, cupric halide selected from a class consisting of cupric bromide and cupric chloride, and a compatible water soluble formate.

2. A photosensitive silver halide print-out emulsion having thereon an overcoating consisting essentially of a water insoluble vinyl acetate polymer emulsion carrier and including as a constituent thereof cupric chloride and

a formate selected from the class consisting of sodium formate, potassium formate, and ammonium formate.

3. A photosensitive silver halide print-out emulsion having thereon an overcoating consisting essentially of a water insoluble vinyl acetate polymeric emulsion carrier and including as a constituent thereof, a cupric halide selected from the class of cupric bromide and cupric chloride, and an alkali metal formate.

4. A photosensitive print-out composition of silver bromoiodide doped with a quantity of cadmium iodide, said composition having thereon an overcoating consisting essentially of a water insoluble vinyl acetate polymeric emulsion carrier having dispersed therein, a cupric halide selected from the class consisting of cupric chloride and cupric bromide, and an alkali metal formate.

No references cited.